

(No Model.)

I. DE V. WARNER & J. C. TALLMAN.

Stiffener for Corsets, &c.

No. 241,100.

Patented May 3, 1881.



Affid  
Courtney & Cooper  
William Paxton.

John C. Tallman  
I. De Ver Warner  
By their attorney  
Charles E. Foster

# UNITED STATES PATENT OFFICE.

IRA DE VER WARNER AND JOHN C. TALLMAN, OF BRIDGEPORT, CONN.

## STIFFENER FOR CORSETS, &c.

SPECIFICATION forming part of Letters Patent No. 241,100, dated May 3, 1881.

Application filed May 19, 1880. (No model.)

*To all whom it may concern:*

Be it known that we, IRA DE VER WARNER and JOHN C. TALLMAN, of Bridgeport, Fairfield county, Connecticut, have invented an Improved Stiffener for Corsets, &c., of which the following is a specification.

The object of our invention is to produce a substitute for the stiffeners or ribs of whalebone and horn heretofore used in corsets, bustles, and other articles of wearing-apparel.

In carrying out our invention we produce a spring-stiffener by binding together a series of straight strips or fibers of "tampico" fiber, which, when confined in bundles of proper size and shape, will constitute flexible elastic substitutes for ordinary stiffening-ribs of whalebone or horn. We have discovered that tampico fibers or stalks when thus bound together form a blade which is stiff, elastic, and as little affected by the heat of the body and perspiration as ordinary bones or horn, and that the blade thus made is a most excellent substitute for whalebone and horn, and much cheaper.

In making such ribs a bundle of tampico stalks, *a*, Figure 1 of the accompanying drawings, may be bound by an outer wrapper formed by binding, plaiting, or braiding threads over the same; or the fibers may be united by metal bands *e*, Figs. 2 and 3, in the form of flat or

round blades. The blades may be flattened by pressure, and, if desired, may be heated, as tampico, when heated, will become tempered and stiffened. This treatment of the fibers, although advantageous and constituting the subject-matter of another application, is not essential, as we make a most effective stiffener by binding the fibers firmly together, and the rib thus formed, which constitutes the subject of this application, has proved to be a most available substitute for the ordinary ribs of whalebone and horn, while costing much less.

We do not here claim the mode of manufacture by pressure between heated surfaces; but

We claim—

As a new article of manufacture, a corset stiffener or rib composed of a series of stiff straight elastic fibers of tampico held together by an external binding, substantially as and for the purposes described.

In testimony whereof we have signed our names to this specification in the presence of two subscribing witnesses.

I. DE VER WARNER.  
JOHN C. TALLMAN.

Witnesses:

G. A. STAPLES,  
P. M. CARY.